

## UNITED STATES PATENT OFFICE

2,223,909

METHOD OF MAKING LAYERS SENSITIVE  
TO LIGHT

Evert Ragnar Elvegård, Stockholm, Sweden

No Drawing. Application March 16, 1938, Serial  
No. 196,286. In Sweden February 11, 1938

2 Claims. (CL 95—7)

It is known to produce light-sensitive layers, using, for example, cellulose as a suspension agent, by successively bathing certain cellulose foils, for example, foils of the kind obtained by 5 the regeneration of cellulose from an aqueous solution of cellulose xanthogenate, so-called viscose foils, in two solutions, containing substances, which after chemical reaction with each other give a precipitate of light-sensitive substances 10 in the foil. Examples of such substances are silver nitrate and potassium bromide, which together give light-sensitive silver bromide.

Further, it is known, when carrying out this method, to use two baths with substances dissolved in water and to give such concentrations to the solutions that the whole quantity of salt absorbed by the foil from the first bath, the so-called impregnation bath, is decomposed when treating the foil in the second bath, which serves 20 as a precipitating agent. The heretofore disclosed method of reaching this result is described to be to keep the molar concentration of the precipitating bath equal to or greater than the molar concentration of the first bath. It has 25 been considered that, if the second bath were molarly more diluted than what has been mentioned above, the precipitate would not be located entirely within the foil but would, at least in parts, form also outside the same in the precipitating bath proper; further, the foil would not 30 possess a smooth and homogeneous appearance.

Yet, films produced in this manner have the drawback of being relatively little light-sensitive, so that considerable times of exposure, also in 35 strong light, are required when they are used for photographic purposes.

The present invention relates to a method of producing light-sensitive layers, which possess a greater light-sensitivity and, therefore, are more 40 useful for various photographic purposes.

The invention is characterized by two moments: 45 (1) The use of at least 3 different solutions; (2) A certain relation between the concentration of the dissolved substances in these solutions. By treating the layer with three or more solutions the advantage is obtained that it is possible to precipitate several different compounds in a certain succession in the layer, which together are able to give a good sensitivity to light 50 to the same.

The concentrations of the different solutions must stand in a definite relation to each other. Investigations have shown that for obtaining a precipitation within the layer and not outside the 55 same, of the insoluble compound the equivalent

normal concentration of a substance in a later used solution must be at least four-tenths of the equivalent-normal concentration of a substance in a previously used solution, with which the first-mentioned substance reacts.

As an example of the use of the invention may be given the precipitation of silver iodide and silver bromide within a viscose foil. In such a case silver iodide should be precipitated first in the foil and then silver bromide. It is possible, however, first to precipitate silver bromide and silver iodide together, but such precipitation should be followed by a precipitation of silver bromide only.

## Example 1

Bath a: 1.0 N. KI  
Bath b: 0.4 N. AgNO<sub>3</sub>  
Bath c: 0.16 N. KBr

## Example 2

Bath a: 1.0 N. KI  
Bath b: 0.4 N. AgNO<sub>3</sub>  
Bath c: 1.0 N. AgNO<sub>3</sub>  
Bath d: 0.4 N. KBr

Examples 1 and 2 state the lowermost limit of the concentration a following bath must have in relation to a previous one. In general, it is, however, advantageous to use a stronger concentration than the said minimum, in accordance with the Examples 3 and 4.

## Example 3

Bath a: 0.1 N. KI  
Bath b: 0.4 N. AgNO<sub>3</sub>  
Bath c: 1.0 N. KBr

## Example 4

Bath a: 0.2 N. AgNO<sub>3</sub>  
Bath b: 0.3 N. KI  
Bath c: 0.6 N. AgNO<sub>3</sub>  
Bath d: 1.0 N. KBr

If, for example, the first bath contains both KI and KBr and the second bath AgNO<sub>3</sub>, which thus reacts with both of the salts in the first bath, the sum of the reacting salts in the first solution is to be counted.

## Example 5

Bath a: 0.2 N. KI+0.3 N. KBr  
Bath b: 0.2 N. AgNO<sub>3</sub>  
Bath c: 0.5 N. KBr.

Analogous is the case, if a following solution contains several substances that react with the substance in a previous solution.

## Example 6

Bath a: 0.8 N. KI  
 Bath b: 1.0 N. AgNO<sub>3</sub>  
 Bath c: 0.3 N. KBr+0.1 N. NaCl.

- 5 According to the invention it is of importance that, if silver iodide is formed in the layer, the same, after the formation of silver iodide has taken place, is treated with a substance influencing the light-sensitivity, which does not consist of nor contains iodine. Preferably, the layer, after the silver iodide is formed, is treated with chlorine or bromine or with a compound containing silver, chlorine or bromine.
- 10 15 For example, a viscose foil is first bathed in a solution obtained by dissolving 0.01 mole potassium iodide in one litre of water. After the foil has been thoroughly impregnated with this solution it is moved to a solution consisting of 0.03 mole silver nitrate in one litre of water, in which case the potassium iodide in the foil will react with penetrating silver nitrate, so that insoluble silver iodide is precipitated within the foil. After the foil has been bathed in the solution of silver nitrate for a suitable length of time, it is removed therefrom and is immersed in a 20 third solution, in which 0.5 mole potassium bromide per litre has been dissolved. Now ions of bromine will penetrate into the foil, where 25 they react with silver nitrate in excess, so that insoluble silver bromide precipitates in the foil. It is left an open question whether this silver bromide is precipitated beside already existing silver iodide or if the former forms mixed crystals or complex compounds with the latter.
- 30 35 A film produced in this manner possesses a considerable sensitivity to light. If, on the other hand, the foil had been treated, for example, first in the solution of potassium bromide, then in the solution of silver nitrate and, finally, in the solution of potassium iodide, a film would have been obtained, the light-sensitivity of which would have been considerably lower.

40 45 As examples of other successions than hereinbefore described for bathing the foil in the solutions the following may be mentioned:

## Example 7



## Example 8



The invention is not restricted only to the halogen silver compounds but is applicable to any 55 silver compounds, for example, organic silver compounds.

The invention is not limited to cellulose foils. It may be applied to any colloids, in or on which 60 light-sensitive silver salts are precipitated by successive treatment with solutions of substances suitable therefor. As examples of colloids, which thus may be used may be mentioned gelatine, casein, dextrose or albumin. A layer consisting of, for example, gelatine, applied to a base 65 of, for example, glass or Celluloid, may thus be made light-sensitive by treatment in solutions of silver salts and halides or other suitable substances.

70 But not even a colloid need be used as a binding agent for the precipitated, insoluble silver salts. For example, by adhesion or adsorption, the same may be fixed to a suitable base. Thus, for example, by combining two solutions, containing silver nitrate and sodium chloride, it is 75 possible to obtain a suitable, disperse precipitate

of silver chloride, which is caused to precipitate on a base, to which the precipitate may be caused to adhere by means of suitable agents. The layer of silver chloride thus obtained may then be treated with solutions of suitable substances, so that other light-sensitive silver salts are precipitated on the same.

75 The treatment of the layer to be made sensitive to light need not be restricted to bathing in solutions of suitable substances. The solutions may, for example, be rubbed or brushed or be pasted on to the layer.

It is possible to sensitize the light-sensitive layers produced according to the invention by using methods or substances customary for sensitizing photographic material. Thus, the light-sensitivity may be increased, if the layer is subjected to a treatment in heat or with an alkaline medium, for example, a solution of ammonia or an organic amine. Also, an increase of the 20 sensitivity is obtained if sulphur-containing sensitizers, for example, thiosinamine, are supplied to the layer. Also, treatment with silver nitrate, which often is used when hyper-sensitizing common photographic film, may be used 25 with advantage on light-sensitive layers produced according to the invention.

In a similar manner the layers may be sensitized for other regions of the spectrum than those of the silver salts by optic sensitizing by 30 means of substances customary for this purpose, such as cyanines, phthaleins, and the like.

For the rest, the foils may be subjected to all treatments, which are customary in the production of common photographic film with gelatine 35 emulsion.

Several light-sensitive layers of different characters may be attached to each other, by which a combined layer may be obtained with desired photographic properties. It is possible also to 40 fasten together one or more prepared layers with one or more unprepared layers of the same material or some other transparent material, for example, of acetate-cellulose or nitro-cellulose.

45 After the treatment in the various baths the layer may be dried either in the air or in a water-absorbing liquid, for example, a water-soluble alcohol, ether, ketone, or aldehyde. In such a case it is advantageous to use easily volatile liquids, the drying being accelerated thereby. The drying by means of a liquid brings about the advantage that the foils dry in a plane state without buckling, which easily may be the case when 55 drying in air. A plane air drying may be obtained also, if the foils, before the drying, are bathed in a solution of glycerine and water.

60 After the drying the surface of the foil presents a glossy, shiny appearance. In certain cases it is, however, desirable that the surface be dull, for example, so as to be able to more easily receive 65 retouching or so as to increase the artistic effect. A dull surface may easily be given to the foil by grinding the surface by means of a powder of a suitable degree of hardness, for example, emery or pumice.

70 The light-sensitive layers produced in accordance with the invention may be used as negative or positive film. It is, however, also possible to fix them to a base of paper or to coat one side of them with a non-transparent, light-reflecting coating, by which the layers may be used for producing pictures for observation in light falling direct on the front side thereof in the same manner as common photographic paper. 75 As examples of a suitable coating may be men-

tioned common white oil-point or white cellulose lacquer. Yet, the base need not be white but may have any shade, for example, ivory or chamois, which shades sometimes may give an increased 5 artistic effect to the picture.

On a suitable occasion during their making the foils may, on one or both sides, be provided with a coating, which is impervious to moisture. As an example of such a coating may be mentioned 10 a colourless transparent nitro-cellulose lacquer.

The invention may be applied with advantage in combination with the object of my application, Serial No. 196,287, filed simultaneously here- 15 with.

Having now described my invention, what I claim as new and desire to secure by Letters Patent is:

1. In a method of making a light sensitive layer using cellulose hydrate as suspension agent 20 by treating the layer with substances, which produce at least one light-sensitive silver com-

pound within the layer, the feature that, after the layer has been subjected to such treatment that silver iodide has been formed, the layer is subjected to a treatment with a solution containing bromide ions but no other halide ions. 5

2. A method of making a light-sensitive layer using cellulose hydrate as suspension agent consisting in at least three successive treatments of the layer with solutions of substances, silver iodide being formed within the layer before the last treatment, the sum of the equivalent-normal 10 concentrations of substances in a later used solution being more than four-tenths of the corresponding sum of substances in a previously used solution with which the first mentioned substances react, the last treatment, after the silver iodide is formed, being performed with a solution, containing bromide ions but no other halide 15 ions.

EVERT RAGNAR ELVEGARD. 20